

## UNITED STATES PATENT OFFICE

2,436,520

## GRAIN REFINING MAGNESIUM ALLOYS

Charles H. Mahoney, Harley C. Lee, Allan L. Tarr,  
and Pierre E. Le Grand, Boulder City, Nev., as-  
signors, by mesne assignments, to Reconstruc-  
tion Finance Corporation, a corporation of the  
United States

No Drawing. Application May 3, 1944,  
Serial No. 533,928

7 Claims. (Cl. 75—67)

1

This invention relates to magnesium alloys and more particularly to magnesium alloys containing aluminum, and has for its object the provision of an improved method of producing such alloys of fine grain structure.

Magnesium alloys, particularly those containing aluminum with or without zinc, when made by customary methods of alloying and refining, inherently solidify in a coarse grain structure. It is now a matter of common knowledge that such magnesium alloys when of fine grain structure possess superior mechanical properties, enhanced amenability to solution treatment, shorter heat-treating requirements, and improved machinability. It is also now a matter of common knowledge that this desirable fine grain structure can be obtained by superheating the molten alloy to temperatures far above the melting temperature of the alloy, as, for example, by superheating at a temperature between 900 and 950° C. The alloy is heated to the superheating temperature, and then cooled to pouring or casting temperature, generally in the neighborhood of 650 to 830° C. This "superheating," as it is called, imparts to the solidified alloy a relatively fine grain structure with the attendant superior properties hereinbefore mentioned. The fine grain structure tends to persist through subsequent remeltings of the alloy, so that castings subsequently produced from superheated alloy possess a fine grain structure.

Superheating of the magnesium alloy is expensive, both on account of the labor and equipment required, and is moreover characterized by uncertainty of duplication and difficulty of control. The temperature required for superheating varies with alloy composition and conditions, and sometimes a superheating temperature giving satisfactory grain refinement with a particular melt may actually give unsatisfactory results when applied to another melt.

We have discovered that carbon-containing substances when introduced into a molten magnesium base alloy at a temperature only slightly above its melting temperature impart to the solidified or subsequently cast alloy a fine-grained structure. Based on that discovery, the present invention involves treating a molten magnesium base alloy with a carbonaceous substance (grain refining agent) which acts on the molten alloy at the temperature of treatment to give the solidified alloy a fine grain structure. The treatment temperature may be only sufficient to maintain the alloy in a molten state, but in practice is preferably somewhat higher, although no advan-

2

tage has been observed with treatment tempera-  
tures in excess of about 800° C. The reaction of  
the carbonaceous material with the molten alloy  
takes place promptly, and treatment periods of a  
few minutes, for example 1 to 15 minutes, are  
satisfactory.

It is our present belief that any organic or  
carbonaceous material in which carbon is re-  
leased or made available in an active form at  
10 the temperature of treatment brings about a  
grain refinement in the solidified alloy. It seems  
likely that the carbon reacts with one of the  
metals of the alloy, probably aluminum in alloys  
15 containing that metal, to form a metal carbide  
which increases the number of grains in the  
solidified structure in contrast with the natural  
coarse-grained structure of castings made from  
the untreated (and non-superheated) alloy.

The carbonaceous grain-refining agent may be  
20 introduced into the molten alloy in gaseous or  
solid, or even liquid, state. Among the carbona-  
ceous substances which may be successfully used  
in practicing the invention are hydrocarbon gases  
25 such as methane, propane and the like, flue gases,  
coal, coke, peat, carbon monoxide, carbon dioxide,  
magnesium carbonate and other carbonates  
which will react with molten magnesium base al-  
loys to give reactive carbon. Air, which contains  
30 some carbon dioxide, even effects some grain re-  
finement, but the action is ineffective in com-  
mercially practical time periods of treatment.  
Similarly, the carbon in graphite and silicon car-  
bide is relatively so inactive that unduly long  
35 periods of treatment are necessary to bring about  
any noteworthy grain refinement. On the other  
hand, propane and other carbonaceous sub-  
stances which are either in whole or in part va-  
porized to give carbon-containing gases at the  
40 temperature of treatment, and which can be in-  
troduced into the molten alloy at the temperature  
of treatment to give reactive carbon, as for ex-  
ample by cracking of the carbonaceous sub-  
stance, may be effectively used in the practice of  
45 the invention. Mixtures of carbonaceous gases,  
such as propane and carbon dioxide, give par-  
ticularly good results.

Most organic substances, including petroleum  
products, coal derivatives, sugars, synthetic plas-  
tics and plant fibers and their derivatives, are  
50 suitable grain-refining agents of the invention.  
In choosing organic substances for the purpose of  
the invention, those yielding high percentages of  
reactive carbon on contacting molten magnesium  
base alloys are most desirable, while those con-  
taining appreciable percentages of chlorine, ni-

trogen, oxygen, sulphur and phosphorous are less desirable. The choice of metallo-organic substances and of carbonates will be governed by economy and by the desire to incorporate or exclude alloying elements which may be natural to the substance. For instance, the use of nickel carbonate would result in contamination of the alloy with metallic nickel which is generally recognized as undesirable because of lessened corrosion resistance of the resulting nickel containing alloy.

Carbon monoxide and carbon dioxide introduced into the molten alloy in gaseous form, or in solid substances which evolve carbon dioxide at the temperature of treatment, are highly effective in achieving grain refinement, but their use is accompanied by the formation of considerable magnesium oxide with incidental metal loss and the necessity of careful subsequent refining of the metal to remove the metal oxide. Treatment with carbon monoxide is preferred to treatment with carbon dioxide because of the lesser amount of oxide formation incident to the use of carbon monoxide. Pulverized coke can be successfully used, but is slower in its action and hence not as desirable as some other sources of carbon. Air (containing carbon dioxide) and flue gas (containing carbon dioxide or carbon monoxide or both and perhaps other carbonaceous gases or substances) require a longer time of treatment to achieve effective grain refinement than does carbon dioxide alone, and moreover result in objectionable nitride and oxide formation, and hence are less desirable grain refining agents of the invention.

The gaseous grain-refining agents of the invention, such for example as propane, may be used in compressed form and bubbled through the molten alloy, in a melting crucible or the like, under sufficient pressure to overcome the molten metal head. Solid agents, such for example as coal or magnesite, are ground or pulverized and added to the molten metal. Where these agents are heavier than the molten magnesium alloy, they will travel downwardly through the molten alloy in a finely disseminated or dispersed condition and thereby effect the necessary contact with the molten alloy. Alternatively, the solid agent may be intimately mixed with the molten alloy by agitation, such as stirring or plunging. In all cases, the surface of the molten alloy may be provided with the usual protective covering, such as a suitable flux or inert gas, to prevent excessive oxidation of the metal. Following the grain refining treatment, it is usually desirable to refine the melt by stirring in a refining flux, as is customary in magnesium refining practice, and separate the small proportion of oxide and other solid and gaseous by-products of the reaction from the molten metal. This cleansing may be aided by allowing the molten metal to remain quiescent for a few minutes before casting. For example, effective elimination of contaminants introduced by the treatment has been achieved in 150 lb. alloy melts by allowing the melt to remain quiescent for 15 minutes at 690° C. prior to casting into ingots.

A surprisingly small quantity of the grain refining agent is adequate for the purposes of the invention. In practice the amount of carbonaceous material required will in general depend upon the reactivity of the carbonaceous material and the degree of dispersion achieved throughout the molten metal. Thus, in the case of solid agents like coal or magnesite, a quantity of the

agent capable of furnishing one percent or less of carbon based on the weight of the magnesium alloy is adequate, and equivalent quantities of gaseous agents are generally adequate. For example, 75 lbs. of propane were sufficient to adequately treat 56,000 lbs. of magnesium alloy, and in another example 10 grams of solid carbonaceous material in the form of pulverized coal were sufficient to satisfactorily treat 150 lbs. of magnesium alloy.

Practice of the invention consistently produces exceptionally fine-grained magnesium alloys which are characterized by initially good mechanical properties which are carried over on subsequent remelting cycles, even though neither re-treatment in accordance with the invention nor superheating is resorted to in such subsequent remelting cycles. However, fine-grained magnesium alloys produced in accordance with the invention can be superheated or retreated in accordance with the invention on the remelt floor without injury. In fact, brief re-treatment in accordance with the invention on the remelt floor tends to quickly establish an optimum fine grain structure so that the quantity of recycled scrap metal on the melting floor becomes unimportant whereas in present practice it is generally considered desirable to add at least 30% of risers, runners and similar scrap to each heat.

The treatment temperature for optimum effectiveness in grain refining is largely dependent on the carbonaceous agent employed. For example in treating a magnesium base alloy with propane at a temperature of 760° C. or slightly lower, maximum grain refinement has been realized in treatment intervals of 2 to 4 minutes, and average grain intercept values of less than 0.0025 inch were obtained in cast ingots. For economy it is desirable to hold the treatment temperature below about 800° C. Heating of the molten alloy to temperatures in excess of that required for achieving maximum grain refinement in accordance with the invention does not impair the effectiveness of the method of the invention, and has no injurious or objectionable effect other than the resulting unnecessary oxidation losses and increased cost.

The invention provides a simple and rapid method of grain refinement permitting the production of fine-grained magnesium alloy structures possessing the properties and characteristics of the fine-grained structures produced by the heretofore customary superheating practices. The grain refinement effected by the invention can be consistently duplicated in successive heats of the same alloy with high regularity in grain size. Thus, the invention enables the consistent production of cast alloys possessing grain sizes smaller than 0.005 inch average intercept value, and, with careful practice, of cast alloys having grain sizes as small as 0.001 inch average intercept value. Like grain refinement by superheating, the invention is particularly applicable to magnesium base alloys containing aluminum, say 2.5 to 10% aluminum, with or without zinc, say 0.2 to 3% zinc. The invention is, however, applicable to all magnesium base alloys capable of responding to present superheating practices to bring about grain refinement, and the invention creates or sets up in the molten alloy a condition that results in the production in the subsequently cast alloy of a very fine-grained structure possessing the properties and characteristics of the fine-grained structure heretofore produced by superheating.

We claim:

1. The method of producing magnesium base alloys of fine grain structure which comprises melting a magnesium base alloy and then treating the molten alloy with a hydrocarbon in which carbon is released in active form at the temperature of treatment.

2. The method of producing magnesium base alloys of fine grain structure which comprises melting a magnesium base alloy and then treating the molten alloy with a hydrocarbon gas.

3. The method of producing magnesium base alloys of fine grain structure which comprises melting a magnesium base alloy and then treating the molten alloy with propane.

4. The method of producing magnesium base alloys of fine grain structure which comprises melting a magnesium base alloy and then treating the molten alloy at a temperature not exceeding about 800° C. with a hydrocarbon in which carbon is released in a form acting on the molten alloy at the temperature of treatment to give a fine grain structure in the subsequent cast alloy.

5. The method of producing magnesium base alloys of fine grain structure which comprises melting a magnesium base alloy and then treating the molten alloy at a temperature not exceeding about 800° C. with a hydrocarbon gas.

6. The method of producing magnesium base alloys of fine grain structure which comprises melting a magnesium base alloy and then treating the molten alloy for a few minutes with a hydrocarbon gas.

7. The method of producing magnesium base alloys of fine grain structure which comprises melting a magnesium base alloy and then treating the molten alloy with an amount of a gaseous

hydrocarbon capable of furnishing upon decomposition in the molten metal up to about 1% of carbon by weight of the molten metal.

CHARLES H. MAHONEY.

HARLEY C. LEE.

ALLAN L. TARR.

PIERRE E. LE GRAND.

#### REFERENCES CITED

10 10 The following references are of record in the file of this patent:

#### UNITED STATES PATENTS

| Number       | Name        | Date          |
|--------------|-------------|---------------|
| 15 1,854,694 | Wood        | Feb. 16, 1932 |
| 1,856,293    | Reitmeister | May 3, 1932   |
| 2,126,786    | Lasch       | Aug. 16, 1938 |
| 2,151,779    | Lasch       | Mar. 28, 1939 |
| 2,380,863    | Nelson      | July 31, 1945 |

#### FOREIGN PATENTS

| Number     | Country | Date         |
|------------|---------|--------------|
| 20 232,581 | Germany | June 7, 1910 |

#### OTHER REFERENCES

- 25 Battelle Memorial Institute, Columbus, Ohio. Reports on Investigation of Cast Magnesium Alloys and of the Existing Foundry Techniques and Practices; Report W-133, published by O. T. S., Apr. 1946; page 43 and pages 1-4 of Preface.
- 30 Ser. No. 387,769, Lepp (A. P. C.) published May 4, 1943.
- Dow, Metals Handbook, 1939 edition, page 1054; published by American Society for Metals.
- 35 Beck, The Technology of Magnesium and its Alloys, published in 1940 by F. A. Hughes and Co., Ltd., Abbey House, N. W. I., London. Page 314.